

# United States Patent Office

2,875,042

Patented Feb. 24, 1959

1

2,875,042

## HIGH TEMPERATURE ALLOY STEEL

Wesley R. Kegerise and Gerald B. Heydt, Reading, Pa., assignors to The Carpenter Steel Company, Reading, Pa., a corporation of New Jersey

No Drawing. Application February 12, 1957  
Serial No. 639,644

11 Claims. (Cl. 75—126)

This invention relates to an alloy steel capable of being age-hardened, having good corrosion resistance, particularly at elevated temperature, and a long stress rupture life with good ductility at elevated temperatures, and to articles made therefrom.

The alloy steel of the present invention is suited for various other uses, but is particularly adapted to meet the ever increasing requirements demanded of turbine parts such as blades, buckets, bolts, etc. Such parts have been subjected to higher and higher operating temperatures and frequently are operated today at temperatures in the range of 800 to 1400° F. To be suitable for such use, the turbine parts must, of course, have good corrosion resistance at these temperatures and because they are subjected to high pressures at these high temperatures, must also have as desirable a stress rupture life as possible. In addition, such an alloy should not become embrittled but should be ductile and retain its ductility under these operating conditions for long periods of time; it should be capable of being annealed so that it can be easily machined at room temperature; and it should be made of reasonably low cost ingredients. Also, the alloy should have a coefficient of expansion which approximates that of the parts to which the alloy is attached, such as the housing, rotors, etc.

In order to achieve as many of these properties as possible, alloy steels have heretofore been used containing around 12% chromium, along with smaller amounts (less than 5%) of one or more other elements such as nickel, tungsten, molybdenum, vanadium and copper, either singly or in combination with one another. Each of these known alloys, however, fails to measure up completely to present day requirements, and has one or more disadvantages. This is particularly true where the alloys are to be subjected to higher temperatures (above 1000° F.) during service. To overcome the shortcomings of these prior alloys at the high temperatures, it has heretofore been necessary to resort to the highly alloyed austenitic alloys, containing large amounts of nickel, cobalt, or amounts of chromium well above 12%. These alloys are extremely expensive, are difficult to fabricate and have a substantially higher coefficient of expansion than the parts to which the components made of these alloys are attached.

It is an object of this invention to provide age-hardenable, inexpensive, essentially ferritic alloys of the 12% chromium steel class, which contain a precipitate in the structure when age hardened, capable of withstanding considerable stress and of high corrosion resistance to steam and the atmosphere at temperatures up to 1400° F., and which are ductile at high temperatures.

It is another object of this invention to provide inexpensive alloys of the 12% chromium steel class, which are essentially ferritic in structure, capable of being age hardened to a value of above Rockwell C-25 subsequent to machining with a minimum of distortion.

2

Other objects of the invention will be apparent to those skilled in the art from reading this specification.

We have found that an alloy can be prepared which meets all of these demands described above to a high degree by incorporating in a 12% chromium steel (i. e., containing about 9-16.5% chromium) certain proportions of molybdenum or tungsten (i. e., about 6-17%). By proper adjustment and control of this composition, a product can be made which after age hardening is essentially ferritic, which has excellent stress rupture characteristics at elevated temperatures, e. g. at 1200° to 1400° F., which is of relatively low cost to manufacture and which can be annealed soft enough for easy machining. For example, such an alloy can be prepared so that it is readily machineable when annealed but can be easily aged to a Rockwell C hardness of above 25. The same alloy, when given a stress rupture test under a 50,000 p. s. i. load at 1200° F., will have a life of at least about 50 hours and frequently as high as 1150 hours. Optional elements including nickel, phosphorus, titanium, vanadium and boron may be added to enhance the properties of the basic alloy.

The composition which has been found to be capable of producing these results is as follows:

|                                                                                  | Percent |
|----------------------------------------------------------------------------------|---------|
| Carbon                                                                           | 10.10   |
| Manganese                                                                        | 1.0     |
| Silicon                                                                          | 1.0     |
| Chromium                                                                         | 9-16.5  |
| Molybdenum and/or tungsten                                                       | 6-17    |
| Balance substantially all iron, except for incidental impurities in such steels. |         |

<sup>1</sup> Maximum.

35 Small residual amounts of phosphorus, vanadium, titanium or boron may be employed singly up to 0.5% phosphorus, 1.0% of vanadium, 0.5% titanium and 0.01% boron to improve the stress rupture properties of the alloy. The optimum amounts of these elements are 0.10% vanadium, 0.05% titanium and about 0.001% boron.

40 The carbon content of the alloy of the invention is desirably limited to 0.1% maximum to insure an essentially ferritic microstructure. It is preferably limited to 0.05%. In the present alloy, carbon is not required for strength. By limiting the carbon to 0.05%, the chromium used for chromium carbide formation is minimized. This increases the amount of chromium available for corrosion resistance and for its effect in insuring an essentially ferritic microstructure.

45 The manganese and silicon contents are desirably limited to 1% maximum. These elements are present solely to provide for deoxidation during melting. Manganese tends to produce an austenitic microstructure and for this reason is desirably limited to 1% maximum.

50 Chromium is necessary in the alloy of the invention for corrosion resistance and it has been established that 9% is required for this purpose. Also below a content of 9% chromium, stress rupture properties are not satisfactory. As chromium content is increased, at the 10% molybdenum level, stress rupture life increases very markedly up to 11.3% chromium and then gradually decreases with further additions up to about 16.5% chromium. Our evaluation based on corrosion resistance and stress rupture life indicates that a 16.5% chromium content represents the desirable maximum limit. We prefer to maintain the chromium content within the range of between about 10 and 14%.

55 Phosphorus is added for its known beneficial effects in strengthening ferrite and improving the stress rupture properties. This improvement can be effected within the

range of 0.1 to 0.50% phosphorus. However, we prefer a range of between about 0.10% and 0.30%, as above this range the addition of phosphorus does not provide a proportionately beneficial increase in stress rupture properties. Phosphorus has the adverse effect of lowering stress rupture ductility, but nickel can be added to overcome this deficiency.

The basic properties of the alloy are substantially improved by the use of 6-17% molybdenum or tungsten. We have found that this controlled amount of molybdenum or tungsten provides an alloy with an essentially ferritic microstructure which surprisingly has excellent resistance to stress rupture at elevated temperatures. Ferrite normally is very soft and ductile, and ferritic steels have not been considered to be good high temperature alloys by those skilled in the art.

We have discovered that the presence of molybdenum and tungsten either separately in amounts of about 6% and above, or together in amounts totaling about 6% and above, improve the stress rupture properties after aging from the annealed condition. These stress rupture properties are much higher than in any other alloy of the ferritic class known to us. The aging reaction provides hardness and strength at elevated temperature, the amount and effect of which is largely controlled by the molybdenum or tungsten content. It is desirable to have a minimum aged hardness of Rockwell C-25. 6% molybdenum will provide the minimum required aged hardness of Rockwell C-25. Amounts of molybdenum above 14% produce increasingly large quantities of one or more intermetallic compounds so that it is difficult to forge the alloys. Additions of molybdenum and/or tungsten over 17% increase the hardness and brittleness due to the increase in the amount of intermetallic compounds so as to render the alloy impractical. The preferred range of molybdenum and/or tungsten is between about 8 and 14%.

Nickel may also be employed in the alloys of the invention. Nickel is added to provide improved stress ruptured ductility. The maximum amount of nickel to be added will vary with the chromium and molybdenum or tungsten additions. The basic alloy is an essentially ferritic alloy and additions of nickel can change it to an austenitic alloy. With lower additions of molybdenum or tungsten and chromium such as 10% each, 4% nickel can be added and still provide an essentially ferritic microstructure. With larger amounts of chromium and molybdenum, the amount of nickel can be raised to a maximum of 6% when the concentrations of chromium and molybdenum or tungsten are at the maximum percentage claimed, and still provide a wholly ferritic alloy.

In order that our invention may be better understood, the following examples of alloy steels prepared according to this invention are given for the purposes of illustration. Percent concentrations of elements in the examples and throughout the specifications are intended to refer to percent by weight, in accordance with the general practice in this art.

*Example I.*—An alloy was prepared having the following analysis:

|            | Percent          |
|------------|------------------|
| Carbon     | 0.022            |
| Manganese  | 0.27             |
| Silicon    | 0.20             |
| Chromium   | 11.3             |
| Molybdenum | 9.9              |
| Phosphorus | 0.218            |
| Boron      | Less than 0.0005 |
| Iron       | Balance          |

The alloy, for test purposes, was cast into 1½ in. square ingots weighing 800 grams each and forged to a ½ in. square bar. The sample showed an essentially ferritic microstructure when annealed by oil quenching from 2000° F. and aged at 1200° F. for 16 hours and had a Rockwell C hardness of 47/48. Samples were

also subjected to stress rupture tests and the results are recorded in the following table:

| Test Temp. | Load, p. s. i. | Percent Elongation in one-inch gauge length | Percent Reduction in Area | Life in Hours |
|------------|----------------|---------------------------------------------|---------------------------|---------------|
| 1,200° F.  | 60,000         | 4.0                                         | 7.6                       | 179.2         |
| 1,200° F.  | 50,000         | 3.8                                         | 6.3                       | 1,152.2       |
| 1,400° F.  | 15,000         | 8.4                                         | 26.8                      | 68.7          |

*Example II.*—An alloy was prepared having the following analysis:

|            | Percent         |
|------------|-----------------|
| Carbon     | 0.034           |
| Manganese  | 0.33            |
| Silicon    | 0.35            |
| Chromium   | 11.4            |
| Molybdenum | 10.0            |
| Phosphorus | 0.194           |
| Boron      | Less than 0.001 |
| Nickel     | 4.07            |
| Iron       | Balance         |

When subjected to the same treatment as specified in Example I, including annealing and aging, the product was essentially ferritic in structure after aging and had a Rockwell C hardness of 46/47. Samples were subjected to stress rupture tests and the results recorded below:

| Test Temp. | Load, p. s. i. | Percent Elongation in one-inch gauge length | Percent Reduction in Area | Life in Hours |
|------------|----------------|---------------------------------------------|---------------------------|---------------|
| 1,200° F.  | 60,000         | 26.6                                        | 57.7                      | 17.6          |
| 1,200° F.  | 50,000         | 13.6                                        | 33.3                      | 103.1         |
| 1,200° F.  | 40,000         | 14.4                                        | 42.0                      | 358.4         |

*Example III.*—An alloy was prepared having the following analysis:

|            | Percent |
|------------|---------|
| Carbon     | 0.024   |
| Manganese  | 0.30    |
| Silicon    | 0.28    |
| Chromium   | 11.21   |
| Molybdenum | 9.96    |
| Nickel     | 0.49    |
| Phosphorus | 0.205   |
| Vanadium   | 0.11    |
| Iron       | Balance |

After being subjected to the same treatment as in Example I, the product was found to have an essentially ferritic microstructure and a Rockwell C hardness of 48. The stress rupture tests under 60,000 p. s. i. at 1200° F. showed a life of 123.2 hours with an elongation in one-inch gauge length of 1% and a reduction in area of 3.4%.

*Example IV.*—An alloy was prepared having the following analysis:

|            | Percent |
|------------|---------|
| Carbon     | 0.032   |
| Manganese  | 0.30    |
| Silicon    | 0.13    |
| Chromium   | 10.86   |
| Molybdenum | 10.04   |
| Nickel     | 0.20    |
| Phosphorus | 0.213   |
| Titanium   | 0.04    |
| Iron       | Balance |

This alloy was subjected to the same treatment as in Example I. It then had a Rockwell C hardness of 48/49. This alloy as aged was essentially ferritic in structure. When subjected to stress rupture tests at

1200° F. under load of 60,000 p. s. i., the samples had a life of 94.2 hours and showed a 4.0% elongation in one-inch gauge length with a reduction in area of 4.7%.

Example V.—An alloy was prepared having the following analysis:

|            | Percent |
|------------|---------|
| Carbon     | 0.038   |
| Manganese  | 0.37    |
| Silicon    | 0.35    |
| Chromium   | 13.22   |
| Molybdenum | 10.16   |
| Phosphorus | 0.187   |
| Iron       | Balance |

When subjected to the same treatment as specified in Example I, the product was essentially ferritic in structure after annealing and aging. Samples were subjected to stress rupture tests at 1200° F. at a load of 60,000 p. s. i. and had a life of 48.3 hours.

Example VI.—An alloy was prepared having the following analysis:

|            | Percent |
|------------|---------|
| Carbon     | 0.022   |
| Manganese  | 0.38    |
| Silicon    | 0.32    |
| Chromium   | 11.46   |
| Molybdenum | 6.8     |
| Phosphorus | 0.222   |
| Iron       | Balance |

After being subjected to the same treatment as in Example I, the product was found to have an essentially ferritic microstructure and a Rockwell C hardness of 37. The stress rupture tests under 50,000 p. s. i. at 1200° F. showed a life of 52.6 hours with an elongation in one-inch gauge length of 6.4% and a reduction in area of 16.7%.

Example VII.—An alloy was prepared having the following analysis:

|            | Percent |
|------------|---------|
| Carbon     | 0.034   |
| Manganese  | 0.33    |
| Silicon    | 0.37    |
| Chromium   | 11.02   |
| Molybdenum | 14.47   |
| Phosphorus | 0.218   |
| Iron       | Balance |

When subjected to the same treatment as specified in Example I, the product was essentially ferritic in structure after annealing and aging and had a Rockwell C hardness of 54/56. Samples were subjected to stress rupture tests and the results recorded below:

| Test Temp. | Load,<br>p. s. i. | Percent<br>Elongation<br>in one-inch<br>gauge length | Percent<br>Reduction<br>in<br>Area | Life in<br>Hours |
|------------|-------------------|------------------------------------------------------|------------------------------------|------------------|
| 1,200° F.  | 60,000            | 1.4                                                  | 3.4                                | 152.9            |
| 1,200° F.  | 50,000            | 1.2                                                  | 3.4                                | 1634.8           |

Example VIII.—An alloy was prepared having the following analysis:

|            | Percent |
|------------|---------|
| Carbon     | 0.034   |
| Manganese  | 0.42    |
| Silicon    | 0.31    |
| Chromium   | 12.6    |
| Molybdenum | 6.97    |
| Tungsten   | 3.08    |
| Phosphorus | 0.204   |
| Iron       | Balance |

After being subjected to the same treatment as in Example I, the product was found to have an essentially

ferritic microstructure and a Rockwell C hardness of 49/51. The stress rupture tests under 60,000 p. s. i. at 1200° F. showed a life of 119.4 hours with an elongation in one-inch gauge length of 2.8% and a reduction in area of 6.3%.

Example IX.—An alloy was prepared having the following analysis:

|            | Percent |
|------------|---------|
| Carbon     | 0.106   |
| Manganese  | 0.37    |
| Silicon    | 0.21    |
| Chromium   | 11.99   |
| Tungsten   | 10.04   |
| Phosphorus | 0.216   |
| Iron       | Balance |

When subjected to the same treatment as specified in Example I, the product was essentially ferritic in structure after annealing and aging. Samples were subjected to stress rupture tests and the results recorded below:

| Test Temp. | Load,<br>p. s. i. | Percent<br>Elongation<br>in one-inch<br>gauge length | Percent<br>Reduction<br>in<br>Area | Life in<br>Hours |
|------------|-------------------|------------------------------------------------------|------------------------------------|------------------|
| 1,200° F.  | 60,000            | 10.0                                                 | 29.3                               | 137.8            |
| 1,200° F.  | 50,000            | 9.2                                                  | 38.3                               | 208.4            |

Example X.—An alloy was prepared having the following analysis:

|            | Percent |
|------------|---------|
| Carbon     | 0.026   |
| Manganese  | 0.27    |
| Silicon    | 0.19    |
| Chromium   | 11.29   |
| Molybdenum | 9.49    |
| Phosphorus | 0.015   |
| Iron       | Balance |

After being subjected to the same treatment as in Example I, the alloy was found to have an essentially ferritic microstructure. The stress rupture tests under 35,000 p. s. i. at 1200° F. showed a life of 1438 hours.

The terms and expressions which we have employed are used as terms of description and not of limitation, and we have no intention, in the use of such terms and expressions, of excluding any equivalents of the features shown and described or portions thereof, but recognize that various modifications are possible within the scope of the invention claimed.

We claim:

1. A steel alloy capable of being age-hardened to show an essentially ferritic structure, said alloy having good corrosion resistance, ductility, impact strength and life at elevated temperatures, and said alloy containing up to about 0.10% carbon, silicon in an amount not more than 1%, manganese in an amount not more than 1%, 9-16.5% chromium, 6-17% of an element selected from the class consisting of molybdenum and tungsten, and the balance iron except for impurities usually associated with these elements.

2. A steel alloy having a structure when aged that is essentially ferritic and having a Rockwell C-scale hardness of above 25, said alloy containing up to about 0.10% carbon, silicon in an amount not more than 1%, manganese in an amount not more than 1%, 9-16.5% chromium, 6-17% of an element selected from the class consisting of molybdenum and tungsten, and the balance principally iron.

3. A turbine part exposed to high temperature and stress, said part consisting of an essentially ferritic alloy having good corrosion resistance, ductility, impact strength and life at elevated temperatures and being readily machineable at room temperature, said alloy containing up to about 0.10% carbon, silicon in an

amount not more than 1%, manganese in an amount not more than 1%, 9-16.5% chromium, 6-17% of an element selected from the class consisting of molybdenum and tungsten, and the balance principally iron.

4. A steel alloy containing carbon up to 0.10%, silicon in an amount not more than 1.0%, manganese up to 1.0%, chromium 9-16.5%, molybdenum 6-17%, and the balance substantially all iron, said alloy having an essentially ferritic microstructure when aged.

5. A steel alloy containing carbon up to 0.10%, silicon and manganese in an amount up to about 1.0% each, chromium 9-16.5%, 6-17% of an element selected from the class consisting of molybdenum and tungsten, up to 0.5% phosphorus, and the balance substantially all iron, said alloy having an essentially ferritic microstructure when aged.

6. A steel alloy containing carbon up to 0.10%, silicon and manganese in an amount up to about 1.0% each, chromium 9-16.5%, 6-17% of an element selected from the class consisting of molybdenum and tungsten, up to 1.0% vanadium, and the balance substantially all iron, said alloy having an essentially ferritic microstructure when aged.

7. A steel alloy containing carbon up to 0.10%, silicon and manganese in an amount up to about 1.0% each, chromium 9-16.5%, 6-17% of an element selected from the class consisting of molybdenum and tungsten, up to 0.5% titanium, and the balance substantially all iron, said alloy having an essentially ferritic microstructure when aged.

8. A steel alloy containing carbon up to 0.10%, silicon and manganese in an amount up to about 1.0% each, chromium 9-16.5%, 6-17% of an element se-

lected from the class consisting of molybdenum and tungsten, up to 0.01% boron, and the balance substantially all iron, said alloy having an essentially ferritic microstructure when aged.

5 9. A steel alloy containing carbon up to 0.05%, silicon up to 1.0%, manganese up to 1.0%, chromium 10-14%, an element selected from the class consisting of tungsten and molybdenum 8-14%, nickel up to 6.0%, and the balance substantially all iron, said alloy having an essentially ferritic microstructure when aged.

10 10. A steel alloy capable of being annealed and aged to give an essentially ferritic structure, said alloy consisting essentially of carbon about 0.022%, silicon about 0.20%, manganese about 0.27%, chromium about 15 11.3%, molybdenum about 9.9%, phosphorus about 0.218%, boron less than 0.0005%, and the balance substantially all iron.

11. A steel alloy capable of being annealed and aged to give an essentially ferritic structure, said alloy consisting essentially of carbon about 0.034%, manganese about 0.33%, silicon about 0.35%, chromium about 16 11.4%, molybdenum about 10%, phosphorus about 0.194%, boron less than 0.001%, nickel about 4.07%, and the balance substantially all iron.

25 References Cited in the file of this patent  
UNITED STATES PATENTS

|           |                |               |
|-----------|----------------|---------------|
| 2,099,509 | Blessing       | Nov. 16, 1937 |
| 2,253,385 | Mahin          | Aug. 19, 1941 |
| 2,289,449 | Nelson         | July 14, 1942 |
| 2,686,116 | Schempp et al. | Aug. 10, 1954 |
| 2,737,455 | Kirkby et al.  | Mar. 6, 1956  |